

# UNITED STATES PATENT OFFICE.

BRADY S. RICHARDSON, OF SCOTTDALE, PENNSYLVANIA.

## FLUX OR SOLUTION FOR COATING METALS.

SPECIFICATION forming part of Letters Patent No. 434,296, dated August 12, 1890.

Application filed April 24, 1889. Serial No. 308,427. (No specimens.)

*To all whom it may concern:*

Be it known that I, BRADY S. RICHARDSON, of Scottdale, in the county of Westmoreland and State of Pennsylvania, have invented a new and improved Flux or Solution for Coating Metals with Lead, of which the following is a full, clear, and exact description.

The object of my invention is to coat articles of iron or other metals with a regular, smooth, and even coating of lead, without previously giving to the metal any coating or galvanizing of other metals for the purpose of preparing them for receiving the lead coating.

15 I will describe my invention as applied to the coating of sheet-iron; but I do not limit or confine myself to this application; as it is equally applicable for coating steel and cast or malleable iron.

20 In carrying out my invention I first clean the sheets of sheet-iron from scale by immersing them in a vat containing dilute sulphuric acid, which is steam-heated to render it more active. I then remove the sheet from

25 the acid and wash it with water. The sheet is then placed in a vat containing water, to which is added lime or other alkaline salts to prevent oxidation and act as a flux. I then put the sheet in a vat containing dilute 30 hydrochloric acid, in which is placed a slab of zinc, upon which the acid acts, forming a solution of chloride of zinc. To this solution are also added certain proportions of oxalic acid, chloride of ammonium, and sulphite of

soda, according to the quantity of material 35 treated. The proportion of oxalic acid and sulphite of soda depends entirely upon the quality of the iron or steel treated; but as an average I use twenty pounds of oxalic acid and ten pounds of sulphite of soda per ton of 40 iron in the dilute hydrochloric acid and zinc bath. After immersion in this solution the sheets are dipped into or passed through melted lead, and as the sheets are withdrawn from the lead a portion of the lead adheres to 45 the surface of the iron, while the surplus drains off into the vat containing the melted metal. The lead thus applied to the sheet of iron forms a very closely-adherent coating, amalgamating with the iron, which resists the action 50 of the atmosphere, and the sheet, while possessing more than the rigidity and strength of iron, has all the advantages of being unoxidable. The use of oxalic acid and sulphite of soda in the bath prevents oxidation and 55 causes a more perfect adhesion of the lead to the iron.

Having thus described my invention, I claim as new and desire to secure by Letters Patent—

60 A solution for the preparation of iron for coating it with lead, said solution consisting of chloride of zinc, oxalic acid, chloride of ammonium, and sulphite of soda, as specified.

BRADY S. RICHARDSON.

Witnesses:

R. W. P. RICHARDSON,  
WILLIAM GIBSON.